

Patented May 24, 1938

2,118,285

# UNITED STATES PATENT OFFICE

2,118,285

## COMPOSITE PERMANENT MAGNETS OF MIXED COMMINUTED ALLOYS

Wilhelm Zumbusch, Krefeld, Germany, assignor  
to Deutsche Edelstahlwerke Aktiengesellschaft,  
Krefeld, Germany, a German company

No Drawing. Application November 7, 1936, Se-  
rial No. 109,683. In Germany November 16,  
1935

7 Claims. (Cl. 175—21)

This invention relates to permanent magnets of the type prepared by pressing finely divided magnetic metal alloy into shapes with or without the use of a binding agent, for example, of 5 a resinous or similar material.

It has been proposed in shaping magnets of the type above described to cast the molten binding agent containing the finely divided magnetic material in suspension. Where a binding 10 agent is not used it has been usual to press the finely divided material in a shell of non-magneteable material.

Permanent magnets of the type above described have been found even with the employment of 15 high pressures in the pressing operation (4 tons per square centimetre or over) to have a density only about 65% of that obtainable when the magnetic material is in the coherent form obtained by casting or rolling the magnetic metal. 20 The consequence of the low specific density of magnets made from finely divided materials, that is to say, its low volumetric fullness factor, is generally a considerable lowering of the remanence of the pressed magnet as compared with 25 a magnet of the same cross section and same composition in the coherent form obtained by casting or rolling. At the same time, the curve fullness factor as expressed by the equation

$$\eta = \frac{BH_{max}}{B_c H_c}$$

in comparison with the coherent material is lowered on an average to the extent of about 30%. The coercive force remains unaltered 35 whether the magnet is in the coherent or finely divided and pressed condition.

In consequence of the above considerations, the available energy per cubic centimetre of a permanent magnet of finely divided material compared with a permanent magnet in coherent condition of the same composition is considerably lower, and reductions have been observed of about 60%. Consequently, for any given purpose a pressed magnet of finely divided material must be made of considerably greater cross section than where a coherent magnet of the same composition is used. This greater cross section is not permissible for many purposes. Even the well-known iron-nickel-aluminium magnetic alloys with their high energy content have not 45 enabled the above-mentioned difficulties to be overcome.

It is an object of this invention to produce 50 magnets consisting of finely divided materials pressed into shape which to a greater extent will be more suitable than those hitherto produced for a variety of purposes, and in particular in such cases in which increased cross section and volume are undesirable owing to restrictions 55 of space in the magnetic system concerned. In

other words, the energy content per cubic centimetre of the pressed magnet of finely divided material must be increased, and the remanence increased to obtain the necessary reduction in magnet cross section. 5

The invention is based on the new discovery that permanent magnets of pressed finely divided material with or without the assistance of a binding agent can be given the most variable properties by employing instead of a single finely divided permanent magnetic material, two or more such materials of different compositions. Both magnetic indices and other properties such as temperature stability and the like may be usefully modified by alteration of the percentage 10 proportions of the ingredients of the mixture. The essential condition for the attainment of special effects by mixing together different permanent magnetic materials is that the coercive force of the ingredients of the mixture should 15 be the same or similar. 20

Conveniently, only such materials are used in which the coercive forces differ by not more than 20% between one material and another. If a material is used in which the coercive force 25 differs by more than 20%, conveniently a special heat treatment should be carried out for one or more materials in order to bring nearer together the values for the coercive forces. The heat treatment consists either in heating and quenching 30 or in the case of precipitation hardenable alloys, to bring about precipitation hardening in any suitable manner.

By suitable mixture of different permanent magnetic materials there is obtained, apart from 35 the advantages which are derived from the pressing process itself, such as easier preparation of complex shapes, the possibility of usefully employing waste material from the preparation of permanent magnets of the most varying kind 40 without the necessity of a remelting process. Materials which are of little use in the pressing process, in particular so far as their remanence 45 and their curve fullness factor is concerned, can be improved by mixing one or more materials which, with approximately the same coercive 50 force, have a higher remanence and a higher curve fullness factor, but which alone are of little use for the preparation of pressed magnets since they contain, for example, large amounts 55 of expensive alloy constituents or they are not obtainable in sufficient quantity in the form of waste material.

Apart from the above-mentioned advantages 60 with regard to magnetic values, by suitable selection of mixture constituents the temperature stability of the finished pressed magnets can be advantageously influenced. In the case of permanent magnetic material with approximately the same magnetic indices the separate materials 65

may, for example, have different temperature stabilities. If then a constituent of lower temperature stability be mixed with a constituent which has the property of temperature stability 5 in a high degree, a pressed magnet is obtained which has a temperature stability which lies between the temperature stability properties of both constituents. The value may be advantageously influenced by the mixture proportions 10 selected.

In the following are given some suitable examples of carrying out the invention:—

For the preparation of a permanent magnet from pressed finely divided material a nickel-aluminium-iron permanent alloy with a coercive force of about 500 oersted, a remanence of about 15 6,000 to 6,500 gauss and a curve fullness factor  $\gamma$  equal to 0.36-0.40 is mixed with a nickel-cobalt-iron permanent magnetic material with a coercive force of 20 500 oersted, a remanence of about 9,000 gauss and a curve fullness factor  $\gamma$  = 0.50, for example, in the proportion of 1:1. The pressed permanent magnet so obtained shows the following values:—B<sub>r</sub> about 4,450 gauss; H<sub>c</sub> about 25 500 oersted;  $\gamma$  about 0.31;

$$\frac{BH_{max}}{8\pi}$$

about 28,000 ergs/cm<sup>3</sup>. Of course, it is possible to 30 use other mixture proportions than 1:1 and thereby attain an extensive modification of the above-mentioned magnetic values.

In the employment of nickel-aluminium-iron for permanent magnetic alloys, materials can 35 also be mixed which have a lower coercive force, for example, 275 oersted in which the remanence comes to 10,000 gauss. This is the case with cobalt-molybdenum-iron permanent magnetic alloys. In order to be able to mix such materials 40 with nickel-aluminium-iron permanent magnetic materials, it is necessary to modify the coercive force of the latter by a special heat treatment consisting of heating and quenching, so that it also has close upon 275 oersted. In consequence 45 of this heat treatment, the magnetic material has a remanence of 8,000 to 8,500 gauss. The curve fullness factor  $\gamma$  for the heat treated nickel-aluminium-iron material comes to 0.5-0.6. With a mixing proportion of 1:1 the above mentioned 50 material gives a permanent magnet with the following values:—B<sub>r</sub> 5550 gauss; H<sub>c</sub> 275 oersted;  $\gamma$  0.36;

$$\frac{BH_{max}}{8\pi}$$

55 22,000 erg/cm<sup>3</sup>.

Carbon - chromium - cobalt - iron permanent magnetic alloys and cobalt-molybdenum-iron alloys have with suitable composition mainly the same magnetic indices, for example, both alloys 60 have a coercive force of about 275 oersted, a remanence of 9,000 to 10,000 gauss. Carbon-chromium-cobalt-iron alloys have the undesired property of being sensitive to temperature influences while the precipitation hardenable permanent magnetic alloys having the basis cobalt-molybdenum-iron are exceptionally insensitive 65 to temperature. By suitable mixing of both alloys, permanent magnets may be obtained which have a considerably better temperature stability 70 than permanent magnets consisting of carbon-chromium-cobalt-iron permanent magnetic alloy alone.

From the examples given it follows that by suitable selection of the constituents to be mixed 75 it is possible without difficulty to prepare per-

manent magnets with every kind of special properties from magnetic materials of known composition in the form of waste, throw outs or the like, so that permanent magnets made of finely divided material with or without binding agents 5 may find a new field, for which hitherto they were not suitable on account of space and reasons of construction.

What I claim is:—

1. Permanent magnets consisting of compressed finely divided magnetic metal alloys, the finely divided material consisting of a mixture of a plurality of different permanent magnetic metal alloys in the finely divided state, the difference between the coercive forces of which is not 15 substantially greater than 20%.

2. Permanent magnets as claimed in claim 1, wherein the finely divided material is united with the aid of a binding agent.

3. Permanent magnets consisting of compressed finely divided magnetic metal alloys, the finely divided material consisting of a mixture of a plurality of different permanent magnetic metal alloys in the finely divided state, wherein a part of the permanent magnetic materials has 25 a high remanence and high curve fullness factor and a part has a low remanence and low curve fullness factor, both parts having approximately the same coercive force, the difference between the coercive forces being not substantially greater than 20%. 30

4. Permanent magnets consisting of compressed finely divided magnetic metal alloys, the finely divided material consisting of a mixture of a plurality of different permanent magnetic metal alloys, wherein the permanent magnetic materials have the same coercive force and remanence, but differ from each other in their sensitivity to temperature influences.

5. A process for the preparation of finely divided permanent magnetic metal alloys for the production of permanent magnets by pressure, characterized in that a plurality of permanent magnetic metal alloys of differing coercive forces are employed, wherein before mixing one or more 40 of the constituent materials is submitted to a heat treatment for the purpose of equalizing the coercive forces, the said heat treatment 45 consisting of heating and quenching the material; and thereafter the constituents are intimately mixed together. 50

6. A process for the preparation of finely divided permanent magnetic metal alloys for the production of permanent magnets by pressure, characterized in that a plurality of permanent magnetic metal alloys of differing coercive forces are employed, wherein before mixing one or more 55 of the constituent materials is submitted to a heat treatment for the purpose of equalizing the coercive forces, the said heat treatment 60 consisting in a precipitation hardening process; and thereafter the constituents are intimately mixed together.

7. A process for the preparation of finely divided permanent magnetic metal alloys for the 65 production of permanent magnets by pressure, characterized in that a plurality of permanent magnetic metal alloys of differing coercive forces are employed, wherein before mixing one or more 70 of the constituent materials is submitted to a heat treatment for the purpose of equalizing the coercive forces, and thereafter the constituents are intimately mixed together. 75